

1

3,211,800

## PROCESS OF DEHYDROGENATION

Laimonis Bajars, Princeton, N.J., assignor to Petro-Tex Chemical Corporation, Houston, Tex., a corporation of Delaware  
No Drawing. Filed Dec. 13, 1962, Ser. No. 244,274  
17 Claims. (Cl. 260—680)

This application is a continuation-in-part of my earlier filed copending and now abandoned application Serial Number 36,718, filed June 17, 1960, entitled, "Dehydrogenation Process."

This invention relates to a process for dehydrogenating organic compounds.

The invention is suitably carried out by passing a mixture, in critical proportions, of the compound to be dehydrogenated, chlorine or a chlorine-liberating compound, and oxygen, at a temperature of at least 450° C., and at an organic compound partial pressure equivalent to less than about one-fifth atmosphere at a total pressure of one atmosphere in the presence of hereinafter defined catalysts, to obtain the corresponding unsaturated organic compound derivative of the same number of carbon atoms.

Suitable hydrocarbons to be dehydrogenated according to the process of this invention are aliphatic hydrocarbons of 4 to 6 carbon atoms and preferably are selected from the group consisting of mono-olefins or diolefins of 4 to 6 carbon atoms, saturated aliphatic hydrocarbons of 4 to 6 carbon atoms and mixtures thereof. Examples of feed materials are butene-1, cis-butene-2, trans-butene-2, 2-methyl butene-3, 2-methyl butene-1, 2-methyl butene-2, n-butane, isobutane, butadiene-1,3, methyl butane, 2-methyl pentene-1, 2-methyl pentene-2 and mixtures thereof. For example, n-butane may be converted to a mixture of butene-1 and butene-2 or may be converted to a mixture of butene-1, butene-2 and/or butadiene-1,3. A mixture of n-butane and butene-2 may be converted to butadiene-1,3 or a mixture of butadiene-1,3 together with some butene-2 and butene-1. n-Butane, butene-1, butene-2 or butadiene-1,3 or mixtures thereof may be converted to vinyl acetylene. The reaction temperature for the production of vinyl acetylene is normally within the range of about 600° C. to 1000° C. such as between 650° C. and 850° C. Isobutane may be converted to isobutylene. The 2-methyl butenes such as 2-methyl butene-1 may be converted to isoprene. Excellent starting materials are the four carbon hydrocarbons such as butene-1, cis or trans butene-2, n-butane, and butadiene-1,3 and mixtures thereof. Useful feeds as starting materials may be mixed hydrocarbon streams such as refinery streams. For example, the feed material may be the olefin-containing hydrocarbon mixture obtained as the product from the dehydrogenation of hydrocarbons. Another source of feed for the present process is from refinery by-products. For example, in the production of gasoline from higher hydrocarbons by either thermal or catalytic cracking a predominantly hydrocarbon stream containing predominantly hydrocarbons of four carbon atoms may be produced and may comprise a mixture of butenes together with butadiene, butane, isobutane, isobutylene and other ingredients in minor amounts. These and other refinery by-products which contain normal ethylenically unsaturated hydrocarbons are useful as starting materials. Another source of feedstock is the product from the dehydrogenation of butane to butenes employing the Houdry process. Although various mixtures of hydrocarbons are useful, the preferred hydrocarbon feed contains at least 50 weight percent butene-1, butene-2, n-butane and/or butadiene-1,3 and mixtures thereof, and more preferably contains at least 70 percent n-butane, butene-1, butene-2 and/or butadiene-1,3 and mixtures thereof. Any remainder usually will be aliphatic hydrocarbons. The process of this invention

2

is particularly effective in dehydrogenating aliphatic hydrocarbons having a straight carbon chain of at least 4 carbon atoms to provide a product wherein the major unsaturated product has the same number of carbon atoms as the feed hydrocarbon.

The chlorine-liberating material may be such as chlorine itself, hydrogen chloride, alkyl chlorides of 1 to 4 carbon atoms such as methyl chloride or ethylene dichloride, carbon tetrachloride, and the like. Preferably the chlorine-containing material will either volatilize or decompose at a temperature of no greater than 100° C. to liberate the required amount of chlorine or hydrogen chloride. Usually an amount of at least 0.01 mol of chlorine per mol of organic compound to be dehydrogenated will be used. It is one of the unexpected advantages of this invention that only very small amounts of chlorine are required. Less than 0.5 mol of chlorine, as 0.2 mol, per mol of organic compound to be dehydrogenated may be employed. Suitable ranges are such as from about 0.01 to 0.05, 0.1 or 0.25 mol of chlorine per mol of the compound to be dehydrogenated. Excellent results are obtained when the chlorine is present in an amount of less than 0.3 mol of chlorine per mol of the compound to be dehydrogenated. It is understood that when a quantity of chlorine is referred to herein, both in the specification and the claims, that this refers to the calculated quantity of chlorine in all forms present in the vapor space under the conditions of reaction regardless of the initial source or the form in which the chlorine is present. For example, a reference to 0.05 mol of chlorine would refer to the quantity of chlorine present whether the chlorine was fed as 0.05 mol of Cl<sub>2</sub> or 0.10 mol of HCl. Preferably the chlorine will be present in an amount no greater than 5 to 10 mol percent of the total feed to the dehydrogenation zone.

The minimum amount of oxygen employed will generally be at least about one-fourth mol of oxygen per mol of organic compound to be dehydrogenated. Large amounts as about 3 mol of oxygen per mol of organic compound may be used. Excellent yields of the desired unsaturated derivatives have been obtained with amounts of oxygen from about 0.4 to about 1.0 or 1.5 mols of oxygen per mol of organic compound and suitably may be within the range of about 0.4 to 2 mols of oxygen per mol of organic compound. Preferably the oxygen will be present in an amount of at least 0.6 mol per mol of compound to be dehydrogenated. Oxygen is supplied to the reaction system as oxygen diluted with inert gases such as helium, carbon dioxide, as air and the like. In relation to chlorine, the amount of oxygen employed should be greater than 1.50 gram mols of oxygen per gram atom of chlorine (or stated differently, this would be greater than 3.0 mols of oxygen per mol of chlorine) present in the reaction mixture. Usually the ratio of the mols of oxygen to the mols of chlorine will be greater than 4 or 5 mols of oxygen per mol of chlorine, such as between 8 and 500 or about 15 and 300 mols of oxygen per mol of chlorine.

The total pressure on systems employing the process of this invention normally will be at or in excess of atmospheric pressure but vacuum may be used. Higher pressures, such as about 100 or 200 p.s.i.g. may be used. The initial partial pressure of the organic compound to be dehydrogenated under reaction conditions is critical and is preferably equivalent to below about one-fifth atmosphere (or about 6 inches of mercury absolute) when the total pressure is atmospheric to realize the advantages of this invention and more preferably equivalent to no greater than 3 or 4 inches of mercury absolute. Also because the initial partial pressure of the hydrocarbon to be dehydrogenated is equivalent to less than about 6 inches of mer-

cury at a total pressure of one atmosphere, the combined partial pressure of the hydrocarbon to be dehydrogenated plus the dehydrogenated hydrocarbon will also be equivalent to less than about 6 inches of mercury. For example, if butene is being dehydrogenated to butadiene, at no time will the combined partial pressure of the butene and butadiene be greater than equivalent to about 6 inches of mercury at a total pressure of one atmosphere. The desired pressure is obtained and maintained by techniques including vacuum operations, or by using helium, organic compounds, nitrogen, steam and the like, or by a combination of these methods. Steam is particularly advantageous and it is surprising that the desired reactions to produce high yields of product are effected in the presence of large amounts of steam. When steam is employed, the ratio of steam to hydrocarbon to be dehydrogenated is normally within the range of about 4 or 5 to 20 or 30 mols of steam per mol of hydrocarbon, and generally will be between 8 and 15 mols of steam per mol of hydrocarbon. The degree of dilution of the reactants with steam, nitrogen and the like is related to keeping the partial pressure of hydrocarbon to be dehydrogenated in the system equivalent to preferably below 6 inches of mercury at one atmosphere total pressure. For example, in a mixture of one mol of butene, three mols of steam and one mol of oxygen under a total pressure of one atmosphere the butene would have an absolute pressure of one-fifth of the total pressure, or roughly six inches of mercury absolute pressure. Equivalent to this six inches of mercury butene absolute pressure at atmospheric pressure would be butene mixed with oxygen and chlorine under a vacuum such that the partial pressure of the butene is six inches of mercury absolute. A combination of a diluent such as steam together with a vacuum may be utilized to achieve the desired partial pressure of the hydrocarbon. For the purpose of this invention, also equivalent to the six inches of mercury butene absolute pressure at atmospheric pressure would be the same mixture of one mol of butene, three mols of steam and one mol of oxygen under a total pressure greater than atmospheric, for example, a total pressure of 15 or 20 inches mercury above atmospheric. Thus, when the total pressure on the reaction zone is greater than one atmosphere, the absolute values for the pressure of butene will be increased in direct proportion to the increase in total pressure above one atmosphere. Another feature of this invention is that the combined partial pressure of the hydrocarbon to be dehydrogenated plus the chlorine-liberating material will also be equivalent to less than 6 inches of mercury, and preferably no greater than 3 or 4 inches of mercury, at a total pressure of one atmosphere. The lower limit of hydrocarbon partial pressure will be dictated by commercial considerations and practically will be greater than about 0.1 inch mercury.

Certain metal elements from the right hand side of the periodic table have been found to act as catalysts for the process and the use of these metal elements is an essential feature of the process. The metal elements which we have found to act as catalysts are selected from the group consisting of copper, zinc, cadmium, aluminum, tin, antimony and bismuth. A variety of active compounds of these metals such as inorganic salts, oxides and hydroxides have been found to be effective in attaining high conversion, selectivity and yield of unsaturated hydrocarbons in accordance with the process of this invention. Materials such as the following may be successfully used in the process of this invention to dehydrogenate hydrocarbons to obtain high yields of unsaturated hydrocarbons: cuprous bromide, cupric bromide, cuprous chloride, cuprous fluoride, cuprous iodide, cuprous oxide, cupric oxide, cuprous silicide, cuprous sulfide, cupric phosphate, elemental zinc, zinc arsenide, zinc borate, zinc fluoride, zinc gallate, zinc oxide, zinc ortho phosphate, zinc phosphide, zinc orthosilicate, zinc metasilicate, zinc sulfide, zinc thiocyanate, aluminum phosphate, aluminum oxide, elemental

5 bismuth, bismuth trioxide, bismuth oxychloride, stannous oxide, stannic oxide, stannous sulfide, elemental antimony, antimony trioxide, antimony tetroxide, cadmium fluoride, cadmium oxide, cadmium orthophosphate, cadmium metasilicate, cadmium sulfate, and the like. Mixtures of the materials and the like in any combination of two or more are also useful.

10 The catalytic metal atoms may be present in various forms such as the elemental metal, or as oxides, salts or hydroxides of the atoms. Many of these metals, salts and hydroxides may change during the preparation of the catalyst, during heating in a reactor prior to use in the process of this invention, or are converted to another form under the described reaction conditions, but such materials still function as an effective compound in the defined process to give increased yields of unsaturated product. Most metals, nitrates, nitrites, carbonates, hydroxides, acetates, sulfites, silicates, sulfides and the like 15 probably converted to the corresponding oxide or chloride under the reaction conditions defined herein. For instance, zinc hydroxide may be charged to the reactor and under the conditions of reaction probably will be converted to zinc oxide. Thus, in the claims and specification when reference is made to the catalyst being a metal compound such as a particular metal oxide or halide, this is intended to include the presence of these oxides or halides regardless of the source; for example, the oxides or halides introduced to the reactor as such or the oxides or halides formed during the course of the reaction would 20 both be included. Such salts as the phosphates, sulfates, halides, some carbonates, and hydroxides and the like, of the defined metal groups, which are normally stable at the defined reaction temperatures are likewise effective under the conditions of the described reaction. Particularly effective in the process of this invention are the defined metals and their oxides, halides and phosphates. In addition, any metal or compound thereof of these groups which are convertible to or are converted under the described reaction conditions to an active catalytic state as the metal, oxide or salt thereof are likewise effective in the process of this invention. Thus, the atoms of the defined catalytic metallic elements are introduced into the reactor in any manner wherein the metallic atoms will be present to catalyze the reaction. Generally the catalytic atoms will be introduced into the reactor as a compound of the metal which, under the conditions of reaction, has a boiling point higher than the temperature of reaction, such as a boiling point of at least 600° C. or 700° C., or 25 may be introduced as a compound which will be converted to a compound which has a boiling point higher than the temperature of reaction. The oxides of the defined metal atoms represent a useful class of materials, since they are inexpensive and are readily formed in situ from metals, salts and hydroxides. Although a great variety of metals 30 and compounds have been found to be useful in the process of this invention, certain of the metals and metal compounds are preferred. Preferred metals and compounds thereof are those of copper, zinc, cadmium, bismuth, antimony, tin, and mixtures thereof, such as the 35 oxides, halides or phosphates of these compounds.

40 The temperature of reaction must be at least 450° C. and preferably will be at least about 500° C. The temperature of the reaction is from about 450° C. to temperatures as high as 850° C. or 1000° C. The optimum temperature is normally determined as by thermocouple at the maximum temperature of the reaction. Usually the temperature of reaction will be from at least or greater than 450° C. to about 750° C. or 900° C. Excellent results have been obtained in the range of about 550° C. to 70 750° C., or 500° C. or 850° C. At the higher temperatures vinyl acetylene may be produced from 4 carbon hydrocarbon feed such as butene or butadiene. The temperatures are measured at the maximum temperature in the reactor.

The flow rates of the gaseous reactants may be varied quite widely and organic compound gaseous flow rates ranging from about 0.1 to about 5 liquid volumes of organic compound per volume of reactor packing per hour have been used. Generally, the flow rates will be within the range of about 0.10 to 25 or higher liquid volumes of the compound to be dehydrogenated, calculated at standard conditions of 0° C. and 760 mm. of mercury per volume of reactor space containing catalyst per hour (referred to as either LHSV or liquid v./v./hr.). Usually the LHSV will be between 0.15 and 15. The volume of reactor containing catalyst is that volume of reactor space excluding the volume displaced by the catalyst. For example, if a reactor has a particular volume of cubic feet of void space, when that void space is filled with catalyst particles the original void space is the volume of reactor containing catalyst for the purpose of calculating the flow rates. The residence or contact time of the reactants in the reaction zone under any given set of reaction conditions depends upon the factors involved in the reaction. Contact times ranging from about 0.001 or 0.01 to about one second or higher such as 10 or 20 seconds have been found to be satisfactory. Residence time is the calculated dwell time of the reaction mixture in the reaction zone assuming the mols of production mixture are equivalent to the mols of feed mixture. For the purpose of calculation of residence times the reaction zone is the portion of the reactor containing catalyst.

For conducting the reaction, a variety of reactor types may be employed. Fixed bed reactors may be used and fluid and moving bed systems are advantageously applied to the process of this invention. In any of the reactors suitable means for heat removal may be provided. Tubular reactors of small diameter may be employed and large diameter reactors which are loaded or packed with packing materials are very satisfactory.

Excellent results have been obtained by packing the reactor with catalyst particles as the method of introducing the catalytic surface. The size of the catalyst particles may vary widely but generally the maximum particles size will at least pass through a Tyler standard screen which has an opening of 2 inches, and generally the largest particles of catalyst will pass through a Tyler screen with one inch openings. Very small particle size carriers may be utilized with the only practical objection being that extremely small particles cause excessive pressure drops across the reactor. In order to avoid high pressure drops across the reactor generally at least 50 percent by weight of the catalyst will be retained by a 10 mesh Tyler standard screen which has openings of  $\frac{1}{16}$  inch. However, if a fluid bed reactor is utilized, catalyst particles may be quite small, such as from about 10 to 300 microns. Thus, the particle size when particles are used preferably will be from about 10 microns to a particle size which will pass through a Tyler screen with openings of 2 inches. If a carrier is used the catalyst may be deposited on the carrier by methods known in the art such as by preparing an aqueous solution or dispersion of the described catalyst, mixing the carrier with the solution or dispersion until the active ingredients are coated on the carrier. The coated particles may then be dried, for example, in an oven at about 110° C. Various other methods of catalyst preparation known to those skilled in the art may be used. When carriers are utilized, these will be approximately of the same size as the final coated catalyst particle, that is, for fixed bed processes the carriers will generally be retained on 10 mesh Tyler screen and will pass through a Tyler screen with openings of 2 inches. Very useful carriers are Alundum, silicon carbide, Carborundum, pumice, kieselguhr, asbestos, and the like. The Alundums or other alumina carriers are particularly useful. When carriers are used, the amount of catalyst on the carrier will generally be in the range of about 5 to 75 weight percent of the total weight of the active catalytic material plus carrier. The carriers

may be of a variety of shapes, including irregular shapes, cylinders or spheres. Another method for introducing the required surface is to utilize as a reactor a small diameter tube wherein the tube wall is catalytic or is coated with catalytic material. If the tube wall is the only source of catalyst generally the tube wall will be of an internal diameter of no greater than one inch such as less than  $\frac{3}{4}$  inch in diameter or preferably will be no greater than about  $\frac{1}{2}$  inch in diameter. Other methods may be utilized to introduce the catalytic surface such as by the use of rods, wires, mesh or shreds and the like of catalytic material. The technique of utilizing fluid beds lends itself well to the process of this invention.

In the above descriptions of catalyst compositions, the composition described is that of the surface which is exposed in the dehydrogenation zone to the reactants. That is, if a catalyst carrier is used, the composition described as the catalyst refers to the composition of the surface and not to the total composition of the surface coating plus carrier. The catalytic compositions are intimate combinations or mixtures of the ingredients. These ingredients may or may not be chemically combined or alloyed. Inert catalyst binding agents or fillers may be used, but these will not ordinarily exceed about 50 percent or 65 percent by weight of the catalytic surface exposed to the reaction gases.

The amount of solid catalyst utilized may be varied depending upon such variables as the activity of the catalyst, the amount of chlorine and oxygen used, the flow rates of reactants and the temperature of reaction. The amount of catalyst will be present in an amount of greater than 25 square feet of catalyst surface per cubic foot of reaction zone containing catalyst. Generally the ratios will be at least 40 square feet of catalyst surface per cubic foot of reaction zone. The catalyst is more effectively utilized when the catalyst is present in an amount of at least 75 square feet of catalyst surface per cubic foot of reaction zone containing catalyst, and preferably the ratio of catalyst surface to volume will be at least 120 square feet of catalyst surface per cubic foot of reaction zone containing catalyst. Of course, the amount of catalyst surface may be much greater when irregular surface catalysts are used. When the catalyst is in the form of particles, either supported or unsupported, the amount of catalyst surface may be expressed in terms of the surface area per unit weight of any particular volume of catalyst particles. The ratio of catalytic surface to weight will be dependent upon various factors including the particle size, particle distribution, apparent bulk density of the particles, amount of active catalyst coated on the carrier, density of the carrier, and so forth. Typical values for the surface to weight ratio are such as about  $\frac{1}{2}$  to 200 square meters per gram,\* although higher and lower values may be used.

The manner of mixing the chlorine or chlorine-liberating compound, organic compound to be dehydrogenated, oxygen containing gas, and steam, if employed, is subject to some choice. In normal operations, the organic compound may be preheated and mixed with steam and preheated oxygen or air, and chlorine or hydrogen chloride are mixed therewith prior to passing the steam in vapor phase over the catalyst bed. Hydrogen chloride or a source of chlorine may be dissolved in water and may be mixed with steam or air prior to reaction. Any of the reactants may be split and added incrementally. For example, part of the chlorine material may be mixed with the hydrocarbon to be dehydrogenated and the oxygen. The mixture may then be heated to effect some dehydrogenation and thereafter the remainder of the chlorine material added to effect further dehydrogenation. The hydrocarbon product is then suitably purified as by frac-

\*As measured by the Innes nitrogen absorption method on a representative unit volume of catalyst particles. The Innes method is reported in Innes, W. B., Anal. Chem., 23, 759 (1951).

tionation to obtain the desired high purity unsaturated product.

In the following examples will be found specific embodiments of the invention and details employed in the practice of the invention. LHSV (or liquid v./v./hr.) means, with reference to the flow rate of organic compound to be dehydrogenated, liquid volume of organic compound per hour per volume of packing or active surface material in the reaction zone. Percent conversion represents mols of organic compound consumed per 100 mols of organic compound fed to a reactor and percent selectivity represents the mols of defined unsaturated organic derivative thereof formed per 100 mols of organic compound consumed. These examples are intended as illustrative only since numerous modifications and variations in accordance with the disclosure herein will be apparent to those skilled in the art. All quantities of chlorine expressed are calculated as mols of  $\text{Cl}_2$ .

*Examples 1 to 4*

A Vycor\* reactor, which was filled with  $\frac{1}{4}$  inch Vycor Raschig rings having deposited thereon the hereinafter designated metal compounds was heated by means of an external electric furnace. The rings were coated with the metal oxides from water slurries thereof and dried before use in a stream of air. At a 700° C. furnace temperature, in a series of runs, butene-2 was used at a flow rate of one liquid v./v./hr. mixed with oxygen and steam at mol ratios of butene to steam to oxygen of 1 to 16 to 0.85. Hydrogen chloride was added as a 37 percent aqueous solution at a rate which was equivalent to 0.115 mol of chlorine ( $\text{Cl}_2$ ) per mol of butene-2. Butene and oxygen were added to the top of the reactor, hydrogen chloride was added to this stream thereafter as it entered the reactor and steam was added separately opposite this stream. The results obtained are in tabular form reported as mol percent conversion, selectivity and yield of butadiene-1,3 per pass.

| Coating            | Percent Conversion | Percent Selectivity | Percent Yield Butadiene-1,3 |
|--------------------|--------------------|---------------------|-----------------------------|
| Bismuth Oxide----- | 64                 | 43                  | 27                          |
| Zinc Oxide-----    | 58                 | 43                  | 25                          |
| Copper Oxide-----  | 85                 | 29                  | 24                          |
| Tin Oxide-----     | 55                 | 43                  | 24                          |

Chlorine is suitably used to replace HCl in these examples. When the above examples are repeated using the same reaction conditions and manganese oxide or ceric oxide on a support as Alundum as a reactor packing, isobutylene is obtained from isobutane and isoprene is obtained from 2-methyl butene-2.

*Example 5*

The run was made in a Vycor reactor which was one inch internal diameter; the overall length of the reactor was about 36 inches with the middle 24 inches of the reactor being encompassed by a heating furnace; the bottom 6 inches of the reactor was empty; at the top of this 6 inches was a retaining plate, and on top of this plate were placed 6 inches of the catalyst particles; the remainder of the reactor was filled with 6 mm. x 6 mm. inert Vycor Raschig rings; the actives of the catalyst were coated on 6 mm. x 6 mm. inert Vycor Raschig rings by depositing a water slurry of the active material on the rings followed by drying overnight at about 110° C., and the flow rates were calculated on the volume of the 6 inch long by 1 inch diameter portion of the reactor which was filled with catalyst particles. The Vycor reactor was packed with Vycor Raschig rings having deposited thereon Fisher A597 aluminum phosphate. At a 700° C. maximum bed temperature, butene-2 was dehydrogenated to butadiene-1,3. The flow rate of butene-2 was

\*Vycor is the trade name of Corning Glass Works, Corning, N.Y., and is composed of approximately 96 percent silica with the remainder being essentially  $\text{B}_2\text{O}_3$ .

5 maintained at  $\frac{1}{2}$  liquid volume of butene-2 (calculated at 0° C. and 760 mm. mercury) per volume of reactor packed with catalyst per hour (l.v./v./hr.). Oxygen and steam were also fed to the reactor in the same stream at a mol ratio of oxygen to butene-2 of 0.85, and a mol ratio of steam to butene-2 of 15. Hydrogen chloride was added to the inlet to the reactor as an aqueous solution at a rate which was equivalent to 0.115 mol of chlorine (calculated as  $\text{Cl}_2$ ) per mol of butene-2. The conversion of butene-2 was 82 mol percent, with 30 mol percent selectivity to butadiene. The resulting yield was 25 mol percent butadiene-1,3 based on the amount of butene-2 fed to the reactor. The catalyst was not coated with carbon.

*Example 6*

10 The procedure for Example 5 was repeated with the exception that the catalyst used was Fisher C-16 cadmium oxide, at 700° C. maximum temperature in the reactor, the conversion was 65, the selectivity was 42 and the yield of butadiene-1,3 was 27.

15 From the foregoing description of the invention, it will be seen that a novel and greatly improved process is provided for producing unsaturated compounds of lower molecular weight but of the same number of carbon atoms as the feed. Other examples could be devised for a process whereby the catalyst contained the described elements; preferably with the described elements constituting greater than or at least fifty atomic weight percent of any cations in the surface exposed to the reaction gases. Although 20 representative embodiments of the invention have been specifically described, it is not intended or desired that the invention be limited solely thereto since it will be apparent to those skilled in the art that modifications and variations may be made without departing from the spirit and scope of the invention. The products such as butadiene-1,3 have many well known uses such as raw materials for the production of synthetic rubber.

I claim:

25 1. The method of dehydrogenating hydrocarbons of 4 to 6 carbon atoms which comprises heating in the vapor phase at a temperature of at least 450° C. an aliphatic hydrocarbon of 4 to 6 carbon atoms with oxygen in a molar ratio of above about one-fourth mol of oxygen per mol of said hydrocarbon, from about 0.01 to less than 0.5 mol of chlorine per mol of said hydrocarbon, the pressure of 30 said hydrocarbon being equivalent to less than about 6 inches of mercury at one atmosphere total pressure with a catalyst comprising a member selected from the group consisting of metals, oxides, hydroxides and salts of copper, zinc, cadmium, tin, antimony, bismuth, and mixtures thereof, the said copper, zinc, cadmium, tin, antimony, bismuth, and mixtures thereof, constituting at least fifty atomic weight percent of any cations in the surface exposed to the reaction gases, the ratio of the mols of said 35 chlorine per mol of said hydrocarbon being greater than 3 mols of oxygen per mol of chlorine.

40 2. The method of claim 1 wherein the said hydrocarbon has four carbon atoms.

45 3. The method of dehydrogenating aliphatic hydrocarbons of 4 to 6 carbon atoms which comprises heating in the vapor phase at a temperature of at least 450° C. the said hydrocarbon with oxygen in a molar ratio of greater than about one-fourth mol of oxygen per mol of said hydrocarbon, chlorine in a molar ratio of about 0.01 to 0.2 mol of chlorine per mol of said hydrocarbon, the initial partial pressure of said hydrocarbon being equivalent to less than about 6 inches mercury at one atmosphere total pressure, with a catalyst comprising a member selected from the group consisting of metals, oxides, hydroxides and salts of copper, zinc, cadmium, tin, antimony, bismuth, and mixtures thereof, the said copper, zinc, cadmium, tin, antimony, bismuth and mixtures thereof, constituting at least fifty atomic weight percent of any cations in the surface exposed to the reaction gases, 50 the ratio of the mols of said oxygen to the mols of said

chlorine being greater than 3 mols of oxygen per mol of chlorine.

4. The method of claim 3 wherein the said hydrocarbon has four carbon atoms.

5. The method of dehydrogenating aliphatic hydrocarbons of 4 to 6 carbon atoms which comprises heating in the vapor phase at a temperature of at least 500° C. a hydrocarbon of 4 to 6 carbon atoms with oxygen in a molar ratio of at least one-fourth mol of oxygen per mol of said hydrocarbon and chlorine in a molar ratio from about 0.01 to less than 0.5 mol of chlorine per mol of said hydrocarbon, the partial pressure of said hydrocarbon being equivalent to less than about 6 inches of mercury at one atmosphere total pressure, with a catalyst comprising a member selected from the group consisting of metals, oxides, hydroxides and salts of copper, zinc, cadmium, tin, antimony, bismuth, and mixtures thereof, the said copper, zinc, cadmium, tin, antimony, bismuth, and mixtures thereof, constituting at least fifty atomic weight percent of any cations in the surface exposed to the reaction gases. The ratio of the mols of said oxygen to the mols of said chlorine being greater than 3 mols of oxygen per mol of chlorine.

6. The method for the production of aliphatic diolefins of 4 to 6 carbon atoms which comprises heating in the vapor phase at a temperature of at least 500° C. the corresponding aliphatic hydrocarbon of 4 to 6 carbon atoms with oxygen in a molar ratio of about 0.4 to 2 mols of oxygen per mol of said aliphatic hydrocarbons, chlorine in a molar ratio of about 0.01 to 0.2 mol of chlorine per mol of said aliphatic hydrocarbons, the partial pressure of said aliphatic hydrocarbons being equivalent to less than about 6 inches mercury at one atmosphere total pressure, with a catalyst comprising a member selected from the group consisting of metals, oxides, hydroxides and salts of copper, zinc, cadmium, tin, antimony, bismuth, and mixtures thereof, the said copper, zinc, cadmium, tin, antimony, bismuth, and mixtures thereof, constituting at least fifty atomic weight percent of any cations in the surface exposed to the reaction gases, the ratio of the mols of said oxygen to the mols of said chlorine being greater than 3 mols of oxygen per mol of chlorine.

7. The method of dehydrogenating aliphatic hydrocarbons of 4 to 6 carbon atoms which comprises heating in the vapor phase at a temperature of at least 450° C. the said hydrocarbon with oxygen in a molar ratio of above about one-fourth mol of oxygen per mol of said hydrocarbon, from about 0.01 to less than 0.5 mol of chlorine per mol of said hydrocarbon, the pressure of said hydrocarbon being equivalent to less than about 6 inches of mercury at one atmosphere total pressure with a catalyst comprising a member selected from the group consisting of oxides of copper, zinc, cadmium, tin, antimony, bismuth, and mixtures thereof, the said copper, zinc, cadmium, tin, antimony, bismuth, and mixtures thereof, constituting at least fifty atomic weight percent of any cations in the surface exposed to the reaction gases, the ratio of the mols of said oxygen to the mols of said chlorine being greater than 3 mols of oxygen per mol of chlorine.

8. The method of claim 7 wherein the said hydrocarbon has four carbon atoms.

9. The method of dehydrogenating aliphatic hydrocarbons of 4 to 6 carbon atoms which comprises heating in the vapor phase at a temperature of at least 450° C. the said hydrocarbon with oxygen in a molar ratio of above about one-fourth mol of oxygen per mol of said hydrocarbon, from about 0.01 to less than 0.5 mol of chlorine per mol of said hydrocarbon, the pressure of said hydrocarbon being equivalent to less than about 6 inches of mercury at one atmosphere total pressure with a catalyst comprising a member selected from the group consisting of salts of copper, zinc, cadmium, tin, antimony, bismuth, and mixtures thereof, the said copper, zinc, cadmium, tin, antimony, bismuth, and mixtures thereof, constituting at least fifty atomic weight percent of any cations in the

surface exposed to the reaction gases, the ratio of the mols of said oxygen to the mols of said chlorine being greater than 3 mols of oxygen per mol of chlorine.

10. The method of claim 9 wherein the said hydrocarbon has four carbon atoms.

11. The method of claim 9 wherein the said salt is a halide.

12. The method for the production of butadiene-1,3 which comprises heating in the vapor phase at a temperature of at least 450° C. n-butene with oxygen in a molar ratio of 0.4 to 1.5 mols of oxygen per mol of n-butene, chlorine in a molar ratio of about 0.01 to 0.2 mol of chlorine per mol of n-butene, and steam in a molar ratio of from 4 to 30 mols per mol of n-butene, with a catalyst comprising a member selected from the group consisting of metals, oxides, hydroxides and salts of copper, zinc, cadmium, tin, antimony, bismuth, and mixtures thereof, the said copper, zinc, cadmium, tin, antimony, bismuth, and mixtures thereof, constituting at least fifty atomic weight percent of any cations in the surface exposed to the reaction gases, the ratio of the mols of said oxygen to the mols of said chlorine being greater than 4 mols of oxygen per mol of chlorine.

13. The method for the production of butadiene-1,3 which comprises heating in the vapor phase at a temperature of at least 500° C. n-butene with oxygen in a molar ratio of 0.40 to 1.5 mols of oxygen per mol of n-butene, chlorine in a molar ratio of between about 0.01 and 0.02 mol of chlorine per mol of said n-butene, the partial pressure of the said n-butene being equivalent to less than about 6 inches of mercury at a total pressure of one atmosphere, with a catalyst comprising copper oxide, the said copper constituting at least fifty atomic weight percent of any cations in the surface exposed to the reaction gases, the ratio of the mols of said oxygen to the mols of said chlorine being greater than 4 mols of oxygen per mol of chlorine.

14. The method for dehydrogenating n-butene which comprises heating in the vapor phase at a temperature of greater than 450° C. n-butene with oxygen in a molar ratio of about 0.4 to 1.5 mols of oxygen per mol of said n-butene, chlorine in a molar ratio of between about 0.01 and 0.2 mol of chlorine per mol of said n-butene, the partial pressure of the n-butene being equivalent to less than about 6 inches of mercury at a total pressure of one atmosphere, with a catalyst comprising zinc oxide, the said zinc constituting at least fifty atomic weight percent of any cations in the surface exposed to the reaction gases, the ratio of the mols of said oxygen to the mols of said chlorine being greater than 4 mols of oxygen per mol of chlorine.

15. The method for dehydrogenating n-butene which comprises heating in the vapor phase at a temperature of greater than 450° C. n-butene with oxygen in a molar ratio of about 0.4 to 1.5 mol of oxygen per mol of said n-butene, chlorine in a molar ratio of between about 0.01 and 0.02 mol of chlorine per mol of said n-butene, the partial pressure of the n-butene being equivalent to less than about 6 inches of mercury at a total pressure of one atmosphere, with a catalyst comprising tin oxide, the said tin constituting at least fifty atomic weight percent of any cations in the surface exposed to the reaction gases, the ratio of the mols of said oxygen to the mols of said chlorine being greater than 4 mols of oxygen per mol of chlorine.

16. The method for dehydrogenating n-butene which comprises heating in the vapor phase at a temperature of greater than 450° C. n-butene with oxygen in a molar ratio of about 0.4 to 1.5 mol of oxygen per mol of said n-butene, chlorine in a molar ratio of between 0.01 and 0.2 mol of chlorine per mol of said n-butene, the partial pressure of the n-butene being equivalent to less than about 6 inches of mercury at a total pressure of one atmosphere, with a catalyst comprising bismuth oxide, the said bismuth constituting at least fifty atomic weight

**11**

percent of any cations in the surface exposed to the reaction gases, the ratio of the mols of said oxygen to the mols of said chlorine being greater than 4 mols of oxygen per mol of chlorine.

17. The method for dehydrogenating n-butene which comprises heating in the vapor phase at a temperature of greater than 450° C. n-butene with oxygen in a molar ratio of about 0.4 to 1.5 mol of oxygen per mol of said n-butene, chlorine in a molar ratio of between 0.01 and 0.2 mol of chlorine per mol of said n-butene, the partial pressure of the n-butene being equivalent to less than about 6 inches of mercury at a total pressure of one atmosphere, with a catalyst comprising cadmium oxide, the said cadmium constituting at least fifty atomic weight percent of any cations in the surface exposed to the re-

5

10

15

**12**

action gases, the ratio of the mols of said oxygen to the mols of said chlorine being greater than 4 mols of oxygen per mol of chlorine.

**References Cited by the Examiner**

## UNITED STATES PATENTS

|           |       |                |       |           |
|-----------|-------|----------------|-------|-----------|
| 2,643,269 | 6/53  | Augustine      | ----- | 260—604   |
| 2,971,995 | 2/61  | Arganbright    | ----- | 260—683.3 |
| 3,028,440 | 4/62  | Arganbright    | ----- | 260—680   |
| 3,116,338 | 12/63 | Guest et al.   | ----- | 260—666   |
| 3,173,962 | 3/65  | Carroll et al. | ----- | 260—659   |

PAUL M. COUGHLAN, *Primary Examiner.*ALPHONSO D. SULLIVAN, *Examiner.*